

W. G. SWART AND B. G. KLUGH.  
PROCESS OF TREATING CONCENTRATES.  
APPLICATION FILED NOV. 17, 1917.

1,303,411.

Patented May 13, 1919.



Witness:

*Conrad Burnap* By *Walter G. Swart*  
*Sheridan, Sheridan & Smith, Atlys* *Bethune G. Klugh*

Inventors:

# UNITED STATES PATENT OFFICE.

WALTER G. SWART, OF DULUTH, MINNESOTA, AND BETHUNE G. KLUGH, OF ANNISTON, ALABAMA.

## PROCESS OF TREATING CONCENTRATES.

1,303,411.

Specification of Letters Patent. Patented May 13, 1919.

Application filed November 17, 1917. Serial No. 202,455.

*To all whom it may concern:*

Be it known that we, WALTER G. SWART, a citizen of the United States, residing at Duluth, in the county of St. Louis and State 5 of Minnesota, and BETHUNE G. KLUGH, a citizen of the United States, residing at Anniston, in the county of Calhoun and State of Alabama, have invented certain new and useful Improvements in Processes 10 of Treating Concentrates, of which the following is a specification.

This invention relates to improvements in processes of treating metalliferous ores, and has for its especial object the preparing of 15 finely divided iron-bearing material, for example, such as concentrates of ores; ores naturally existing as very fine sand, earth, dust, or clay, or artificial ores; or by-products carrying iron values, for sintering or 20 other agglomerating processes, and also natural or artificial ores requiring desulfurization, dehydration, or elimination of any volatile constituents by volatilization of such constituents.

25 Finely divided or clayey iron-bearing materials, require some form of agglomeration before they can be efficiently treated in blast furnaces. Agglomeration by such blast roasting processes as the Heberlein, the 30 Dwight and Lloyd, and the Greenawalt, for instance, requires, first, that the finely divided or clayey iron-bearing material to be agglomerated shall be intimately and thoroughly mixed with solid fuel, preferably 35 carbonaceous and finely divided, prior to its delivery to the blast roasting or sintering apparatus; and, second, that such mixture of solid fuel and finely divided or clayey iron-bearing material be delivered to such 40 sintering apparatus containing a definite percentage of water or other fluid, which so "tempers" it, or brings it to such a state of plasticity, that it contains the largest possible volume or percentage of voids, which is 45 desirable for best sintering practice.

It happens that much of the finely divided and clayey iron-bearing material occurring naturally and the concentrates made artificially contain approximately the right 50 amount of moisture to give them the proper degree of plasticity, or can be brought easily to this condition, but it also happens that this condition or degree of plasticity is that at which it is most difficult to secure the 55 necessary intimate mixture of the material

or concentrate with the solid fuel. The 60 gummy, sticky nature of the mass is such as to interfere seriously with the successful operation of any mixing device now in use, requiring a heavy excess of power, giving 65 much trouble from breakage of machine parts, necessitating frequent stopping of machines for cleaning out caked and packed masses, and delivering a product imperfectly mixed.

65 In the case of the pug mill or blade type of mixer, the plastic material builds up into hard cakes on all surfaces adjacent to the peripheral path of the blades, thus causing a braking action on the blades with enormously increased power consumption and 70 wear on the blades. In the case of the drum or cylindrical type of mixer the gummy material builds up on all surfaces with which it comes in contact, forming cakes or masses 75 difficult to dislodge, causing an excess power consumption, reducing the mixing area and volume of the apparatus, and giving poor mixing. At intervals the mixers must be 80 stopped and cleaned or all mixing stops. Such finely divided iron-bearing materials as fine magnetite concentrates, now being extensively produced, and ores naturally plastic, such as those Cuban ores known as Mayarri ores, are especially productive of difficulty and expense as just described.

85 By our invention we propose to eliminate the mixing devices as above described with their attendant difficulties and expense.

When finely divided ore is concentrated 90 on tables, or in magnetic and other separators, the concentrates are customarily delivered from the concentrating machines in a semi-fluid condition, due to the excess of water contained therein. This excess of water must be removed before sintering, and this removal may be effected in several ways, but filtering machines of the Oliver or Portland type offer a desirable method.

95 In our process the finely divided fuel, which if necessary has been previously crushed or ground, while either dry or wet, in suitable machines such as ball mills, is introduced into the fluid mass of concentrates and thoroughly mixed therewith by 100 any suitable means, such as a centrifugal pump, while the concentrates are still fluid; and the excess water is then removed by any suitable apparatus, such as a revolving filter, 105 which delivers a plastic mass with the fuel 110

already intimately mixed therewith, and in the best physical condition for sintering, without further mixing.

In the case of a sticky, gummy, or clayey ore occurring naturally, like the Mayari Cuban ores already mentioned, we vary our process only by first adding sufficient water to the natural ore to bring it to a semi-fluid condition, then adding the finely divided fuel, as before, then thoroughly agitating and mixing the semi-fluid mass and filtering same to the desired degree of plasticity. It has heretofore been found impossible to get a suitable mixture of fuel with this kind of ore to allow good sintering except at a prohibitive cost.

Certain (natural) ores and by-products (natural or artificial) contain sulfur, combined water, or other volatile constituents, to an amount which renders them undesirable, or even totally unfit, for blast furnace use. When such ores occur massive they do not require agglomeration for the purpose of keeping fines out of the blast furnace, but for the equally necessary purpose of removing the objectionable elements mentioned. It is therefore necessary to crush such ores and sinter them, which sintering not only eliminates the fines, but at the same time removes these objectionable elements. Such procedure is now being followed commercially at several plants. The practice is to grind the ore dry, add the necessary fuel, moisten to sintering consistency in the mixer, then sinter the mass. Wet grinding is preferable, but not used, because an excess of water must be added which would have to be subsequently removed by drying, leaving the same sort of plastic mass as described above, with which it is difficult to mix the necessary fuel.

Under the invention described herein, such ores may be ground wet, have the necessary fuel added and mixed while the mass is still fluid, then filtered and sintered, as already described.

The fuel may be added to such ore previous to, or simultaneous with, or subsequent to, the grinding of the ore, the mixed ore and fuel being then filtered and sintered.

Iron-bearing ore and other products are sometimes leached for the removal of copper, zinc, or other substances, either in a natural state or subsequent to roasting. Such leached material is usually plastic and difficult to mix with fuel for subsequent sintering. By our method, water is added until the mass is fluid. Fuel is then added and easily mixed, the resulting mixture being filtered and sintered, as herein described.

As a further feature of this invention, we contemplate the use of peat, which to our knowledge has not heretofore been used as a fuel in sintering or otherwise agglomerating ores. Peat usually occurs naturally in such

form that it must be macerated and dried before being used as fuel. It is not uncommon for it to be taken from the bogs carrying 75% to 80% water, most of which it is difficult and expensive to remove. In our invention we introduce the peat into the semi-fluid mass of concentrates or ore, without necessarily drying the peat, then agitate and mix the semi-fluid mass of ore or concentrates and peat, and then filter the fluid 75 mass, the result being a plastic mass containing the necessary fuel intimately mixed, ready for sintering, just as though finely divided coal or coke, or other solid fuel, had been used.

Peat often occurs in swamps in a naturally semi-fluid condition. Our invention also covers the inverted procedure of introducing the finely divided iron-bearing materials into the fluid or pulpy peat, and then subjecting the mixture to a filtering or dewatering operation, substantially as described, before agglomeration.

It is evident that in the case of fuels other than peat, also, it makes no difference in the 90 final result whether the ore is added to the fuel or the fuel to the ore, either or both being in the same liquid pulpy condition, or in the dry state.

To illustrate one method of carrying out 95 our process, we have shown one form of apparatus in the accompanying drawing, in which—

A designates a crushed ore bin or hopper from which the finely crushed ore is delivered to a concentrator indicated by B, the embodiment shown being of the type known as the "Davis" type, in which the ore is magnetically separated and at the same time conveyed to the upper end of the concentrator, where it is discharged in the form of a pulp or fluid mass into the launder C. Located above the latter is a bin D, in which is located the fuel in the desired condition, such as peat, comminuted or ground to desired condition, a feed roller D' being located beneath the open end thereof to deliver the fuel in desired proportion to the launder C, as indicated by dotted lines. A valve D<sup>2</sup> may be utilized to control the amount of 115 fuel delivered. This fuel, together with the fluid pulp, flows through the medium of the launder C<sub>1</sub> and C<sub>2</sub> to a centrifugal pump E, where the fuel and fluid ore particles are thoroughly mixed and commingled and delivered through the conduit E' to a filtering machine, generally indicated by the letter F, and shown as of the Oliver or Portland type, the excess moisture being pumped out by the filtering machine in a manner well 120 known to those skilled in the art, and the de-watered mixture of ore and fuel is carried over on the lip or chute F' to the feeding hopper G which is located above the endless belt H' of a sintering apparatus, for 125 130

example, generally indicated by the letter H. A slide valve G' may be used to regulate the delivery of the mixture to the sintering belt H<sub>1</sub>. The apparatus for sintering 5 shown here is of the Dwight and Lloyd type, although as in the case of the apparatus diagrammatically illustrated in the drawing, we do not wish to be restricted to any specific type or form of apparatus in the 10 carrying out of this process. H<sub>2</sub> indicates the suction box of the sintering apparatus through the medium of which combustion is carried through the mixture after ignition thereof and during the passage of the 15 exhaust box H<sub>2</sub>.

It will be apparent that, by the addition of the fuel in the manner and at the time described, a thorough homogeneity of the mixture is obtained with a minimum of 20 labor and expense by utilizing a necessary step in the handling of the concentrates.

It will be obvious that while the carrying 25 out of our process in the above-described apparatus delivers the comminuted ore in a pulpy or fluid condition so as to flow readily, it is possible that we may treat fine or plastic ores by reducing them to a fluid or pulpy condition previous to the mixture of the fuel therewith.

30 Further modifications and changes in our process as described are possible and contemplated, and we do not wish to be restricted to the herein-described process save as defined in the appended claims.

35 What we claim is:

1. A process of the class described com-

prising the steps of mixing fuel and metalliferous particles with water to obtain a fluid mixture, then removing the excess water content, and then agglomerating the 40 mixture.

2. A process of the class described comprising the steps of mixing fuel with metalliferous particles in a fluid state, then removing the excess water content, and then 45 agglomerating the mixture.

3. A process of the class described, consisting in first mixing metalliferous particles of desired size with water or the like, to a state of fluidity, then adding fuel, next 50 mixing said fuel and fluid, then removing superfluous water content, and finally agglomerating said mixture.

4. A process of the class described, consisting in first mixing metalliferous particles of the desired size with water or the like to a state of fluidity, then adding peat thereto, next mixing said peat and metalliferous fluid, then removing superfluous water content from said mixture, and finally 55 60 agglomerating the same.

In testimony whereof, we have subscribed our names.

WALTER G. SWART.

Witnesses:

T. B. COUNSELMAN,  
H. N. MACHAIG.

BETHUNE G. KLUGH.

Witnesses:

W. O. J. KOPP,  
W. E. NICHOLIS.